# EUROPEAN PATENT SPECIFICATION

(11) **EP 0 155 131 B1**
(45) Date of publication and mention of the grant of the patent: **08.08.1990**
(21) Application number: 85301462.9
(22) Date of filing: 05.03.1985
(51) Int. Cl.: C10M 169/06

(54) **Grease composition containing boron compound and hydroxy containing soap thickener**
Eine Borverbindung und eine hydroxy-substituierte Seife als Verdickungsmittel enthaltende Fettzusammensetzung
Composition de graisse contenant un composé de bore et un savon contenant un substituant hydroxyle comme agent épaississant

(30) Priority: 07.03.1984 US 587328; 15.08.1984 US 641077
(43) Date of publication of application: 18.09.1985
(73) Proprietor: MOBIL OIL CORPORATION, New York New York 10017 (US)
(72) Inventor: Doner, John Phillips, Sewell New Jersey 08080 (US); Horodysky, Andrew Gene, Cherry Hill New Jersey 08003 (US); Keller, John Antone, Jr., Pitman New Jersey 08071 (US)
(74) Representative: Cooper, John Anthony

(56) References cited:
- GB-A- 1 400 020
- GB-A- 2 102 023
- GB-A- 2 106 133
- GB-A- 2 125 431
- US-A- 3 125 523
- US-A- 3 125 524
- US-A- 3 125 525
- US-A- 4 328 113
- US-A- 4 382 006

## Description

The invention is concerned with the novel group of compositions. It more particularly relates to a synergistic grease composition comprising oil, hydroxy-containing soap thickener and borated amine, and optionally containing phosphorus and sulfur moieties.

US Patents, 3125523; 3125524 and 3125525 disclose lubricating greases thickened with hydroxy fatty acid soaps and comprising salts formed from amines and borate esters.

The present invention seeks to provide lubricating greases of improved dropping point.

According to one aspect of this invention, there is provided an improved grease composition which comprises:
i. a major proportion of a grease vehicle;
ii. thickener which contains at least 15% by weight of a hydroxy-containing soap thickener; and
iii. from 0.01 % to 10% by weight of a condensation product made by reacting boric acid with an amine of the formula: wherein:
   x is 0 to 2;
   R, R', R³ or R⁴, which may be the same or different, each represents a hydrogen atom or a C, to C₃₀ hydrocarbyl group, a C_{z} to C₄ hydroxyalkyl group, a C₆ to C₂₀ polyalkoxylated group which may comprise sulfur or additional oxygen, with the proviso that at least one of R, R¹, R³ or R4 does not represent a hydrogen atom; and R represents a C₂ to C₄ alkylene group.

The presence of a phosphorus and sulfur moieties provides an even higher dropping point. The alkyl borates include the mono-, di- and trialkyl borates, i.e., those having the methyl, ethyl, propyl, butyl, pentyl and hexyl groups.

Preferably the amine is overborated. By "overborated" is meant the presence in the borated product of more than a stoichiometric amount of boron with respect to the amine.

Included within the scope of the amines as set forth in the above formula are (1) the primary amines such as hexylamine, octylamine, nonylamine, decylamine, dodecylamine, tetradecylamine, octadecylamine, eicosylamine, triacontylamine, oleylamine, stearylamine, isostearylamine, tallowamine and soyamine, (2) the secondary amines corresponding to (1) having both groups the same or having mixtures of such groups, (3) the corresponding tertiary amines where again all the groups in the same molecule can be the same or different and (4) diamines such as N-octyl-1,2-ethylenediamine or the N-octyl-1,3-propylenediamine, N-coco-1,2-ethylenediamine or the N-coco-1,3-propylenediamine, N-oleyl-1,2-ethylenediamine, or N-oleyl-1,3-propylenediamine, N-soya-1,2-ethylenediamine or the N-soya-1,3-propylenediamine and N-tallow-1,2-ethylenediamine or the N-tallow-1,3-propylenediamine. The secondary amines include N-ethyl-N-oleylamine, N-methyl-N-soyamine, and the tertiary amines include N,N-diethyl-N-oleylamine.

Alkoxylated amines included are bis(2-hydroxyethyl)olelylamine, bis(2-hydroxypropyl)oleylamine, bis(2-hydroxyethyl)tallowamine, bis(2-hydroxypropyl)tallowamine, (hydroxyethyl)(hydroxypropyl)tallowamine, polyethoxylated oleylamine (containing 7 ethoxy groups) and polyethoxylated tallowamine (containing 3 ethoxy groups). Included also are hydroxyalkyl amines made by the ethoxylation or propoxylation of hydrocarbyldiamines or hydrocarbyltriamines. Specifically included are aromatic or alkyl-or alkylene-substituted aromatic groups containing 6 to 30 carbon atoms. Further included are alkoxyalkylamines, such as dodecyloxypropylamine and triisodecyloxypropylamine and similar oxygen- containing amines, and the corresponding alkoxydiamines, such as the N-alkoxyhydrocarbylenediamines.

The reaction to form the condensation product (iii) can be carried out at from about 80°C to about 260°C, preferably from about 110°C to about 180°C. The temperature chosen will depend for the most part on the particular reactants and on whether or not a solvent is used. Reaction pressures can be vacuum, atmospheric or positive pressure. In carrying out this reaction, it is preferable that quantities of reactants be chosen such that the molar ratio of amine to boric acid be from about 0.2 to about 2, preferably from about 0.5 to about 0.9. The amine can be reacted with an excess of the boric acid to form a condensation product containing from about 0.1% by weight of boron to as much as 10% or more of boron.

While atmospheric pressure is generally preferred, the reaction can be advantageously run at from about 1 to about 5 atmospheres. Furthermore, where conditions warrant it, a solvent may be used. In general, any relatively non-polar, unreactive solvent can be used, including benzene, toluene, xylene and 1,4-dioxane. Other hydrocarbon and alcoholic solvents, which include propanol, butanol, hexamethylene glycol and the like, can be used. Mixtures of alcoholic and hydrocarbon solvents can also be used.

The times for the reactions are not critical. Thus, any phase of the process can be carried out from about 1 to about 20 hours.

A narrow class of thickening agents is preferred to make the grease of this invention. Included among the preferred thickening agents are those containing at least a portion of alkali metal, alkaline earth metal or amine soaps of hydroxy-containing fatty acids, fatty glycerides and fatty esters having from 12 to about 30 carbon atoms per molecule. The metals are typified by sodium, lithium, calcium and barium. Preferred is lithium. Preferred members among these acids and fatty materials are 12-hydroxystearic acid and glycerides and esters containing 12-hydroxystearates, 14-hydroxystearic acid, 16-hydroxystearic acid and 6-hydroxystearic acid.

The entire amount of thickener need not be derived from the aforementioned preferred members. Significant benefit can be attained using as little thereof as about 15% by weight of the total thickener. A complementary amount, i.e., up to about 85% by weight of a wide variety of thickening agents can be used in the grease of this invention. Included among the other useful thickening agents are alkali and alkaline earth metals soaps of methyl-12-hydroxystearate, diesters of a C₄ to C₁₂ dicarboxylic acid and tall oil or marine oil fatty acids. Other alkali or alkaline earth metal fatty acids containing from 12 to 30 carbon atoms and no free hydroxyl may be used. These include soaps of stearic and oleic acids.

Other thickening agents include salt and salt-soap complexes as calcium stearate-acetate (U.S. Patent No. 2,197,263), barium stearate acetate (U.S. Patent No. 2,564,561), calcium, stearate-caprylate-acetate complexes (U.S. Patent No. 2,999,065), calcium carpylate-acetate (U.S. Patent No. 2,999,066) and calcium salts and soaps of low-, intermediate- and high-mblecular weight acids of nut oil acids.

Another group of thickening agents comprises substituted ureas, phthalocyamines, indanthrene, pigments such as perylamides, pyromellitdiimides, and ammeline, as well as certain hydrophobic clays. These thickening agents can be prepared from clays which are initially hydrophilic in character, but which have been converted into a hydrophobic condition by the introduction of long-chain hydrocarbon radicals into the surface of the clay particles prior to their use as a component of a grease composition, as, for example, by being subjected to a preliminary treatment with an organic cationic surface active agent, such as an onium compound. Typical onium compounds are tetraalkylammonium chlorides, such as dimethyl dioctadecyl ammonium chloride, dimethyl dibenzyl ammonium chloride and mixtures thereof. This method of conversion, being well known to those skilled in the art, is believed to require no further discussion, and does not form a part of the present invention.

Manufacture of the thickening agents can be done in a variety of grease making equipment such as in open kettles at reduced, atmospheric, or positive pressures; in higher pressure reaction chambers which may be operated to as high as 180 psig; or in continuous manufacturing equipment. The temperature range from the bulk grease under manufacture can range from 15°C (60°F) to 238°C (460°F).

The third member(s) that may be present in the grease composition are the phosphorus and sulfur moities. Both of these can be present in the same molecule, such as in a metal or non-metal phosphorodithioate of the formula wherein R⁶ is a hydrocarbyl group containing 3 to 18 carbon atoms, M is a metal or non-metal, n is the valence of M and Z is oxygen or sulfur, at least one Z being sulfur.

In this compound, R⁶ is preferably an alkyl group and may be a propyl, butyl, pentyl, hexyl, octyl, decyl, dodecyl, tetradecyl or octadecyl group, including those derived from propanol, isopropanol, butanol, isobutanol, sec-butanol, 4-methyl-2-pentanol, 2-ethylhexanol, oleyl alcohol, and mixtures thereof. Further included are alkaryl groups such as butylphenyl, octylphenyl, nonylphenyl and dodecylphenyl groups.

The metals covered by M include those in Groups IA, IIA, IIB and VIII of the Periodic Table. Some that may be mentioned are lithium, molybdenum, sodium, calcium, zinc, cadmium, silver and gold. Non- metallic ions include organic groups derived from vinyl esters such as vinyl acetate, vinyl ethers such as butyl vinyl ether, epoxides such as propylene oxide and 1,2-epoxydodecane and amine salts. They also include other nitrogenous compounds such as those derived from hydrocarbyl amines and diamines, including oleylamine and N-oleyl-1,3-propylenediamine and such as the imidazolines and oxazolines.

The phosphorus and sulfur can also be supplied from the combination of two separate compounds, such as the combination of (1) a dihydrocarbyl phosphite having 2 to 10 carbon atoms in each hydrocarbyl group or mixtures of phosphites and (2) a sulfide such as sulfurized isobutylene, dibenzyl sulfide, sulfurized terpenes, phosphorodithionyl disulfide and sulfurized jojoba oil. The phosphites embrace the dibutyl, dihexyl, dioctyl, didecyl and similar phosphites. Phosphate esters containing 4 to 20 carbon atoms in each hydrocarbyl group, such as tributyl phosphate, tridecyl phosphate, tricresyl phosphate and mixtures of such phosphates, can also be used.

In summary, it is essential to the practice of this invention, in which greases having vastly improved dropping points are obtained, that at least the first two of the above-mentioned ingredients be formulated into the composition. Thus:
first, with respect to the preparation of the grease, the thickener will have at least about 15% by weight of a metal or non-metal hydroxy-containing soap therein, the total thickener being from about 3% to about 20% by weight of the total grease composition;
second, there will be added to the grease from about 0.01 % to about 10% by weight, preferably about 0.1 % to about 2%, of a condensation product, in which an amine, has been reacted with, preferably, at least an equimolar amount of boric acid and
as an optional third component, the composition may have therein from 0.01% to about 10% by weight, preferably from 0.2% to 2% by weight, of a compound containing both phosphorus and sulfur moieties or a mixture of two or more compounds which separately supply the phosphorus and sulfur moieties. If separate compounds are used, an amount of the mixture equivalent to the above concentration levels is used to supply desired amounts of phosphorus and sulfur.

It was noted that, when the hydroxy-containing thickener was used with the condensation product (iii), the dropping point of the grease was consistently unexpectedly higher than a grease from the same grease vehicle and the same reaction product, but with a different thickener, e.g., a non-hydroxy-containing thickener. Thus, the broad invention is to a grease composition comprising the two components mentioned.

In general, the reaction products of the present invention may be employed in any amount which is effective for imparting the desired degree of friction reduction, antiwear activity, antioxidant activity, high temperature stability or antirust activity. In many applications, however, the condensation product (iii) and the phosphorus- and/or sulfur-containing compound(s) are effectively employed in combined amounts of from about 0.02% to about 20% by weight, and preferably from about 0.2% to about 4% of the total weight of the composition.

The greases of the present invention can be made from either a mineral oil or a synthetic oil, or mixtures thereof. In general, mineral oils, both paraffinic, naphthenic and mixtures thereof, may be of any suitable lubricating viscosity range, as for example, from about 45 SSU at 100°F to about 6000 SSU at 100°F, and preferably from about 50 to about 250 SSU at 210°F. These oils may have viscosity indexes ranging up to about 100 or higher. Viscosity indexes from about 70 to about 95 are preferred. The average molecular weights of these oils may range from about 250 to about 800. In making the grease, the lubricating oil from which it is prepared is generally employed in an amount sufficient to balance the total grease composition, after accounting for the desired quantity of the thickening agent, and other additive components to be included in the grease formulation.

In instances where synthetic oils are desired, in preference to mineral oils, various compounds of this type may be successfully utilized. Typical synthetic vehicles include polyisobutylene, polybutenes, hydrogenated polydecenes, polypropylene glycol, polyethylene glycol, trimethylol propane esters, neopentyl and pentaerythritol esters, di(2-ethylhexyl) sebacate, di(2-ethylhexyl) adipate, dibutyl phthalate, fluorocarbons, silicate esters, silanes, este'f's of phosphorus-containing acids, liquid ureas, ferrocene derivatives, hydrogenated synthetic oils, chain-type polyphenyls, siloxanes and silicones (polysiloxanes), alkyl-substituted diphenyl esters typified by a butyl-substituted bis(p-phenoxy phenyl) ether, phenoxy phenylethers.

The metallic soap grease compositions containing one or more of the borated amines, and optionally, one or more of the sulfur and phosphorus combinations described herein provide advantages in increased dropping point, improved grease consistency properties, antirust characteristics and potential antifatigue, antiwear and antioxidant benefits unavailable in prior greases. The grease of this invention is unique in that it can be preferably manufactured by the admixture of additive quantities of the alcohol borates to the fully formed soap grease after completion of saponification.

The following Examples illustrate the invention.

### Example 1

A mixture of 1295 g of N-oleyl-1,3-propylenediamine (obtained as Duomeen O from Armak Chemical Co.), 218 g of xylene, 437 g of n-butanol, 658 g of hexamethylene glycol and 1210 g of boric acid were placed in a reactor equipped with heater, agitator and Dean-Stark tube with condenser, and refluxed for about 10 hours until all water formed in the reaction azeotroped over (maximum temperature was about 195°C). The solvents were removed by vacuum distillation at 195°C and the product was filtered and then diluted with an equal amount of 100 second process oil to form a 50% concentrate of borated diamine in mineral oil. The concentrate was an orange colored viscous liquid.

### Example 2

N-tallow-1,3-propylenediamine (obtained as Duomeen T obtained from Armak Chemical Co.) was borated with boric acid as generally described in Example 1. For convenience of handling, the borated N-tallow-1,3-propylenediamine was blended with an equal wt. of 100 second process oil to form a 50% concentrate in mineral oil.

### Example 3

A lithium hydroxystearate grease thickener was prepared by saponification of a mixture containing 12-hydroxystearic acid (8%) and the glyceride thereof (9%) with lithium hydroxide in a mineral oil vehicle at about 177°C in a closed contactor.

### Example 4

After depressuring and dehydration of the thickener in an open kettle, sufficient mineral oil was added to reduce the thickener content to about 9.0%. After cooling to about 99°C, a typical grease additive package, consisting of an amine antioxidant, phenolic antioxidant, metallic dithiophosphate (1.5 wt.% of zinc dialkyl phosphorodithioate, where the alkyl is derived from a mixture of C₃ to C₆ primary alcohols), sulfur-containing metal deactivator and nitrogen containing antirust additives, was added.

### Example 5

To the base grease of Example 4, was added at about 110°C, 0.5 wt.% of the borated N-oleyl-1,3-propylenediamine of Example 1.

### Example 6

To the base grease of Example 4, was added at about 115°C, 1.0 wt.% of the borated N-tallow-1,3-propylenediamine of Example 2.

### Example 7

To the base grease of Example 3 was added 0.5 wt.% of the borated N-oleyl-1,3-propylenediamine of Example 1.

### Example 8

Same as Example 7, except 2% of borated amine was used.

### Example 9

Base grease thickened with the lithium soap of 50/50 (wt) mixture of stearic and palmitic acids, which are non-hydroxy-containing thickeners.

### Example 10

50 wt.% of the base grease used in Example 4 plus 50 wt.% of the grease of Example 9, producing a 50-50 mixture of hydroxy- and non-hydroxy-containing thickeners.

### Example 11

Base grease of Example 9 containing 2 wt.% of the borated amine of Example 2.

Results obtained in the ASTM D2265-78 grease dropping point test are shown in the following table.

Examples 5 and 6 show a significant effect upon dropping point improvement when borated amine is added to hydroxy-containing carboxylate soap thickened grease in the presence of a phosphorus and sulfur source.

Examples 7 and 8 show a significant effect upon hydroxy-containing carboxylate soap thickened grease when the borated amines described are used.

Examples 9, 10 and 11 clearly show no benefit of the borated amine upon the dropping point of a non-hydroxy-containing carboxylate soap thickened grease.

## Claims

1. An improved grease composition which comprises:
i. a major proportion of a grease vehicle;
ii. thickener which contains at least 15% by weight of a hydroxy-containing soap thickener; and
iii. from 0.01 % to 10% by weight of a condensation product made by reacting boric acid with an amine of the formula: wherein:
x is 0 to 2;
R, R', R³ or R⁴, which may be the same or different, each represents a hydrogen atom or a C₁ to C₃₀ hydrocarbyl group, a C₂ to C₄ hydroxyalkyl group, a C₆ to C₂₀ polyalkoxylated group which may comprise sulfur or additional oxygen, with the proviso that at least one of R, R', R³ or R⁴ does not represent a hydrogen atom; and R² represents a C₂ to C₄ alkylene group.

2. A composition according to Claim 1 additionally containing from about 0.01% to about 10% by weight of a compound containing both phosphorus and sulfur moieties or a mixture of phosphorus-containing and sulfur-containing compounds to supply an equivalent amount of phosphorus and sulfur.

3. A composition according to Claim 1 or 2 wherein the thickener is an alkali metal, alkaline earth metal or amine soap of a hydroxyl-containing fatty acid, fatty glycerine or fatty ester containing 12 to 30 carbon atoms.

4. A composition according to Claim 3 wherein the metal is sodium, lithium, calcium or barium.

5. A composition according to any preceding claim wherein the thickener is derived from 12-hydroxystearic acid, 14-hydroxystearic acid, 16-hydroxystearic acid, 6-hydroxystearic acid or the glyceride or ester thereof.

6. A composition according to any preceding claim wherein R, R¹, R³ or R⁴, which may be the same or different, each represents a hydrogen atom or a C₆ to C₂₀ alkyl group with the proviso that at least one of R, R', R³ or R" does not represent a hydrogen atom.

7. A composition according to any preceding claim wherein the amine is (1) hexylamine, octylamine, nonylamine, decylamine, dodecylamine, tetradecylamine, octadecylamine, eicosylamine, triacontylamine, oleylamine, stearylamine, isostearylamine, tallowamine, soyamine, (2) the secondary amines corresponding to (1) having both groups the same or having mixtures of such groups, (3) the corresponding tertiary amines wherein all the groups in each molecule are the same or different, or (4) N-octyl-1,2-ethylenediamine, N-octyl-1,3-propyleneamine, N-coco-1,2-ethylenediamine, N-coco-1,3-propylenediamine, N-oleyl-1,2-ethylenediamine, N-oleyl-1,3-propylenediamine, N-soya-1,2-ethylenediamine, N-soya-1,3-propylenediamine, N-tallow-1,2-ethylenediamine, N-tallow-1,3-propylenediamine, N-ethyl-N-oleylamine, N-methyl-N, soyamine, N,N-diethyl-N,oleylamine, bis(2-hydroxyethyl)oleylamine, bis(2-hydroxypropyl)oleylamine, bis-(2-hydroxy)tallowamine, bis(2-hydroxypropyl-tallowamine, (hydroxyethyl)(hydroxypropyl)tallowamine, polyethoxylatedoleylamine containing 7 ethoxy groups, polyethoxylated tallowamine containing 3 ethoxyl groups, hydroxyalkyl amines made by the ethoxylation or propoxylation of hydrocarbyldiamines or hydrocarbyltriamines, dodecyloxypropylamine or triisodecyloxypropylamine.

8. A composition according to any preceding claim wherein the phosphorus and sulfur moeities are supplied by a phosphorothioate of the formula wherein R⁶ is a hydrorcarbyl group containing 3 to 18 carbon atoms, M is a metal or non-metal, n is the valence of M and Z is oxygen or sulfur, at least one Z being sulfur.

9. A composition according to Claim 8 wherein R⁶ is an alkyl group or an alkaryl group.

10. A composition according to Claim 9 wherein R⁶ is a propyl, butyl, pentyl, octyl, dodecyl, tetradecyl, octadecyl, butylphenyl, octylphenyl, nonylphenyl dodecylphenyl or oleyl group or a mixture thererof.

11. A composition according to Claim 10 wherein R⁶ is derived from propanol, isopropanol, butanol, isobutanol, sec-butanol, 4-methyl-2-pentanol, 2-ethylhexanol or a mixture thereof.

12. A composition according to any of claims 8 to 11 from Group IA, IIA, IIB or VIII of the Periodic Table.

13. A composition according to Claim 12 wherein the metal is lithium, sodium, silver, molybdenum, calcium, zinc, cadmium or gold.

14. A composition according to any of Claims 8 to 11 wherein M is derived from vinyl acetate, butyl vinyl ether, propylene oxide, 1,2-epoxydodecane or nitrogenous compound.

15. A composition according to any of Claims 1 to 7 wherein the phosphorus and sulfur moieties are supplied by a combination of (1) a dihydrocarbyl phosphite having 2 to 6 carbon atoms in each hydrocarbyl group, mixtures of such phosphites, or a phosphate ester having 4 to 20 carbon atoms in each hydrocarbyl group and (2) a sulfide selected from sulfurized isobutylene, dibenzyl disulfide, sulfurized terpenes, phosphorodithionyl disulfide and sulfurized jojoba oil.

16. A composition according to Claim 15 wherein the phosphite is a dibutyl, dihexyl, dioctyl or didecyl phosphite or mixtures thereof.

17. A composition according to Claim 15 wherein the phosphate ester is a tributyl, tridecyl or tricresyl phosphate or mixtures thereof.

18. A composition according to Claim 1 wherein the amine is N-oleyl-1,3-propylenediamine, the thickener is 2-hydroxystearate and the phosphorus and sulfur are supplied by zinc C₃ to C₆ alkyl phosphorodithioate.

19. A composition according to Claim 1 wherein the amine is N-tallow-1,3-propylenediamine, the boron compound is boric acid, the thickener is lithium 12-hydroxystearate and the phosphorus and sulfur moieties are supplied by zinc C₃ to C₆ alkyl phosphorodithioate.

20. A composition according to any preceding claim wherein the grease vehicle is a mineral oil.

21. A composition according to any preceding claims wherein the grease vehicle is a synthetic oil.

22. A composition according to Claim 20 and 21 wherein the grease vehicle is a mixture of mineral and synthetic oils.

23. A composition according to any preceding claim wherein the total amount of the thickener is from about 3% to about 20% by weight of the total grease composition.

24. A method of improving the dropping point of a grease composition comprising a major proportion of a grease vehicle and from about 0.01% to about 10% by weight of a condensation product made by reacting boric acid with an amine of the formula wherein:
x is 0 to 2;
R, R¹, R³ or R⁴ are hydrogen or hydrocarbyl groups containing from 1 to 30 carbon atoms, hydroxyalkyl groups containing 2 to 4 carbon atoms, a polyalkoxylated group containing 6 to 20 carbon atoms or the latter group containing sulfur or additional oxygen, at least one of R, R', R³ or R" being a non-hydrogen group and R is a C₂ to C₄ alkylene group with a boron compound, said method comprising thickening said grease with a thickener containing at least 15% by weight of a hydroxy-containing soap thickener.

25. A method according to Claim 24 in which the grease composition additionally contains from about 0.01% to about 10% by weight of a compound containing both phosphorus and sulfur or a mixture of phosphorus-containing and sulfur-containing compounds to apply an equivalent amount of phosphorus and sulfur.

## Patentansprüche

1. Verbesserte Schmierfettzusammensetzung aus
i. einem Hauptanteil eines Schmierfetträgers,
ii. einem Verdickungsmittel, das wenigstens 15 Gew.-% einer hydroxylgruppenhaltigen Seife als Verdickungsmittel enthält, und
iii. 0,01 bis 10 Gew.-% eines Kondensationsprodukte, das durch Umsetzung von Borsäure mit einem Amin der Formel hergestellt wurde, worin
x eine Zahl von 0 bis 2 ist,
R, R¹, R³ oder R⁴, die gleich oder verschieden sein können, jeweils ein Wasserstoffatom oder einem Cᵢ- bis C30-Kohlenwasserstoffrest, einen C₂- bis C₄-Hydroxyalkylrest oder einen C₆- bis C₂₀-polyalkoxylierten Rest, der Schwefel oder zusätzlichen Sauerstoff enthalten kann, bedeuten, mit der Maßgabe, daß wenigstens einer der Reste R, R', R³ oder R⁴ kein Wasserstoffatom ist, und R^{I} einen C₂- bis C₄-Alkylenrest darstellt.

2. Zusammensetzung nach Anspruch 1, die zusätzlich etwa 0,01 bis etwa 10 Gew.-% einer Verbindung enthält, die sowohl phosphor- als auch schwefelhaltige Rest oder ein Gemisch aus phosphorhaltigen und schwefelhaltigen Verbindungen enthält, um eine äquivalente Menge an Phosphor und Schwefel zur Verfügung zu stellen.

3. Zusammensetzung nach Anspruch 1 oder 2, worin das Verdickungsmittel eine Alkalimetall-, Erdalkalimetall- oder Aminseife einer hydroxylgruppenhaltigen Fettsäure, eines Glycerins mit Fettsäureresten oder eines Fettsäureesters mit 12 bis 30 Kohlenstoffatomen ist.

4. Zusammensetzung nach Anspruch 3, worin das Metall Natrium, Lithium, Calcium oder Barium ist.

5. Zusammensetzung nach der einem vorhergehenden Ansprüche, worin das Verdickungsmittel von 12-Hydroxystearinsäure, 14-Hydroxystearinsäure, 16-Hydroxystearinsäure, 6-Hydroxystearinsäure oder einem Glycerid oder Ester davon abgeleitet ist.

6. Zusammensetzung nach einem der vorhergehenden Ansprüche, worin R, R', R³ oder R⁴, die gleich oder verschieden sein können, jeweils ein Wasserstoffatom oder eine C₆- bis C₂₀-Alkylgruppe darstellen, mit der Maßgabe, daß wenigstens einer der Reste R, R', R³ oder R⁴ kein Wasserstoffatom darstellt.

7. Zusammensetzung nach einem der vorhergehenden Ansprüche, worin das amin (1) Hexylamin, Octylamin, Nonylamin, Decylamin, Dodecylamin, Tetradecylamin, Octadecylamin, Eicosylamin, Triacontylamin, Oleylamin, Stearylamin, Isostearylamin, Talgamin oder Sojamin ist, (2) ein (1) entsprechendes sekundäres Amin ist, das entweder zwei gleiche Reste oder Gemische solcher Reste aufweist, (3) ein entsprechendes tertiäres Amin ist, worin alle Reste in jeweils einem Molekül gleich oder verschieden sind, oder (4) N-Octyl-1,2-ethylendiamin, N-Octyl-1,3-propylendiamin, N-Kokos-1,2-ethylendiamin, N-Kokos-1,3-propylendiamin, N-Oleyl-1,2-ethylendiamin, N-Oleyl-1,3-propylendiamin, N-Soja-1,2-ethylendiamin, N-Soja-1,3-propylendiamin, N-Talg-1,2-ethylendiamin, N-Talg-1,3-propylendiamin, N-Ethyl-N-oleylamin, N-Methyl-N-sojamin, N,N-Diethyl-N-oleylamin, Bis-(2-hydroxyethyl)-oleylamin, Bis-(2-hydroxypropyl)-oleylamin, Bis-(2-hydroxyethyl)-talgamin, Bis-(2-hydroxypropyl)-talgamin, (Hydroxyethyl)-(hydroxypropyl)-talgamin, polyethoxyliertes Oleylamin mit 7 Ethoxygruppen, polyethoxyliertes Talgamin mit 3 Ethoxygruppen, Hydroxyalkylamine, die durch Ethoxylierung oder Propoxylierung von Kohlenwasserstoffdiaminen oder Kohlenwasserstofftriaminen hergestellt wurden, Dodecyloxypropylamin oder Triisodecyloxypropylamin, ist.

8. Zusammensetzung nach einem der vorhergehenden Ansprüche, worin die phosphor- und schwefelhaltigen Reste durch ein Phosphorthioat de Formel zur Verfügung gestellt werden, worin R⁶ ein Kohlenwasserstoffrest mit 3 bis 18 Kohlenstoffatomen, M ein Metall oder ein Nichtmetall, n die Wertigkeit von M und Z Sauerstoff oder Schwefel ist, wobei wenigstens ein Z Schwefel ist.

9. Zusammensetzung nach Anspruch 8, worin R⁶ ein Alkyl- oder Alkarylrest ist.

10. Zusammensetzung nach Anspruch 9, worin R⁶ ein Propyl-, Butyl-, Pentyl-, Hexyl-, Octyl-, Dodecyl-, Tetradecyl-, Octadecyl-, Butylphenyl-, Octylphenyl-, Nonylphenyl-, Dodecylphenyl- oder Oleylrest oder ein Gemisch davon ist.

11. Zusammensetzung nach Anspruch 10, worin R⁶ von Propanol, Isopropanol, Butanol, Isobutanol, sek.-Butanol, 4-Methyl-2-pentanol, 2-Ethylhexanol oder einem Gemisch davon abgeleitet ist.

12. Zusammensetzung nach einem der Ansprüche 8 bis 11, wobei M ein Metall aus der Gruppe IA, IIA, IIB oder VIII des Periodensystems ist.

13. Zusammensetzung nach Anspruch 12, worin das Metall Lithium, Natrium, Silber, Molybdän, Calcium, Zink, Cadmium oder Gold ist.

14. Zusammensetzung nach einem der Ansprüche 8 bis 11, worin M von Vinylacetat, Butylvinylether, Propylenoxid, 1,2-Epoxydodecan oder einer stickstoffhaltigen Verbindung abgeleitet ist.

15. Zusammensetzung nach einem der Ansprüche 1 bis 7, worin die phosphor- und schwefelhaltigen Reste durch eine Kombination von (1) einem Dihydrocarbylphosphit mit 2 bis 6 Kohlenstoffatomen in jedem Kohlenwasserstoffrest, Gemischen solcher Phosphite oder einem Phosphatester mit 4 bis 20 Kohlenstoffatomen in jedem Kohlenstoffrest, und (2) einem Sulfid, ausgewählt aus der Gruppe sulfuriertes .Isobutylen, Dibenzyldisulfid, sulfurierte Terpene, Phosphordithionyldisulfid und sulfuriertes Jojobaöl, zur Verfügung gestellt werden.

16. Zusammensetzung nach Anspruch 15, worin das Phosphit ein Dibutyl-, Dihexyl-, Dioctyl- oder Didecylphosphit oder ein Gemisch davon ist.

17. Zusammensetzung nach Anspruch 15, worin der Phosphatester ein Tributyl-, Tridecyl- oder Tricresylphosphat oder ein Gemisch davon ist.

18. Zusammensetzung nach Anspruch 1, worin das Amin N-Oleyl-1,3-propylendiamin und das Verdickungsmittel 12-Hydroxystearat ist sowie der Phosphor und Schwefel durch Zink-C₃- bis C₆- alkylphosphordithioat zur Verfügung gestellt werden.

19. Zusammensetzung nach Anspruch 1, worin das Amin N-Talg-1,3-propylendiamin, die Borverdindung Borsäure und das Verdickungsmittel Lithium-12-hydroxystearat ist sowie die phosphor-und schwefelhaltigen Reste durch Zink-C₃- bis C6-alkylphosphordithioat zur Verfügung gestellt werden.

20. Zusammensetzung nach einem vorhergehenden Ansprüche, worin der Schmierfettträger ein Mineralöl ist.

21. Zusammensetzung nach einem vorhergehenden Ansprüche, worin der Schmierfettträger ein synthetisches Öl ist.

22. Zusammensetzung nach Anspruch 20 und 21, worin der Schmierfettträgir ein Gemisch aus Mineralöl und synthetischem Öl ist.

23. Zusammensetzung nach einem der vorhergehenden Ansprüche, worin die Gesamtmenge des Verdickungsmittels etwa 3 bis 20 Gew.-% der gesamten Schmierfettzusammensetzung beträgt.

24. Verfahren zur Verbesserung des Tropfpunkts einer Schmierfettzusammensetzung, enthaltend einen Hauptanteil eines Schmierfettträgers und etwa 0,01 bis etwa 10 Gew.-% eines Kondensationsprodukts, das durch Umsetzung von Borsäure mit einem Amin der Formel hergestellt wurde, worin x eine Zahl von 0 bis 2 ist, R, R', R³ oder R⁴ Wasserstoffatome oder Kohlenwasserstoffreste mit 1 bis 30 Kohlenstoffatomen, Hydroxyalkylreste mit 2 bis 4 Kohlenstoffatomen oder einen polyalkoxylierten Rest mit 6 bis 20 Kohlenstoffatomen bedeuten oder der letztere Rest Schwefel oder zusätzlichen Sauerstoff enthält, wobei wenigstens einer der Reste R, R¹, R³ und R⁴ kein Wasserstoffatom ist, und R^{Z} einen C_{z}- bis C₄-Alkylenrest mit einer Borverbindung darstellt, wobei das Verfahren das Verdicken des genannten Schmierfetts mit einem Verdickungsmittel, das wenigstens 15 Gew.-% einer hydroxylgruppenhaltigen Seife als Verdickungsmittel enthält, beinhaltet.

25. Verfahren nach Anspruch 4, bei dem die Schmierfettzusammensetzung zusätzlich etwa 0,01 bis etwa 10 Gew.-% einer Verbindung enthält, die sowohl Phosphor als auch Schwefel oder ein Gemisch von phosphorhaltigen und schwefelhaltigen Verbindungen, die eine äquivalente Menge an Phosphor und Schwefel zur Verfügung stellen, enthält.

## Revendications

1. Une composition de graisse améliorée, caractérisée en ce qu'elle comprend:
i. une proportion majeure d'une graisse servant de véhicule;
ii. un agent épaississant qui contient au moins 15% en poids d'un savon ayant un substituant hydroxy en tant qu'agent épaississant; et
iii. de 0,01% à 10% en poids d'un produit de condensation obtenu par réaction d'acide borique avec une amine de formule: dans laquelle
x a une valeur de 0 à 2;
R, R', R³ ou R⁴ qui peuvent être identiques ou différents, représentent chacun un atome d'hydrogène ou un groupe hydrocarbyle en C₁₋₃₀, un groupe hydroxyalkyle en C₂₋₄, un groupe polyalcoxylé en ce C₆-_{zo} pouvant comprendre du soufre ou de l'oxygène supplémentaire, à condition qu'au moins l'une des R, R', R³ ou R⁴ ne soit pas un atome d'hydrogène; et R² représente un groupe alkylène en C₂-₄.

2. Une composition suivant la revendication 1, caractérisée en ce qu'elle contient de plus d'environ de 0,01 à 10% en poids d'un composé contenant à la fois des entités phosphore et soufre, ou d'un mélange de composés contenant du phosphore et contenant du soufre pour fournir une quantité équivalente de phosphore et de soufre.

3. Une composition suivant les revendications 1 ou 2, caractérisée en ce que l'agent épaississant est un savon de métal alcalin, métal alcalino-terreux ou d'amine d'un acide gras, glycéride gras ou ester gras ayant un substituant hydroxy, contenant 12 à 30 atomes de carbone.

4. Une composition suivant la revendication 3, caractérisée en ce que le métal est le sodium, le lithium, le calcium ou le baryum.

5. Une composition suivant l'une quelconque des revendications 1 à 4, caractérisée en ce que l'agent épaississant provient de l'acide 12-hydroxystéarique, de l'acide 14-hydroxystéarique, de l'acide 16-hydroxystéarique, de l'acide 6-hydroxystéarique ou du glycéride ou d'un ester de ceux-ci.

6. Une composition suivant l'une quelconque des revendications 1 à 5, caractérisée en ce que R, R', R³ ou R⁴ qui peuvent être identiques ou différents, représentent chacun un aome d'hydrogène ou un groupe alkyle en C₆₋₂₀, à condition qu'au moins l'un des R, R', R³ ou R⁴ ne soit pas un atome d'hydrogène.

7. Une composition suivant l'une quelconque des revendications 1 à 6, caractérisée en ce que l'amine est (1) l'hexylamine, l'octylamine, la nonylamine, la décylamine, la dodécylamine, la tétradécylamine, l'octadécylamine, l'éicosylamine, la triacontylamine, l'oléylamine, la stéarylamine, l'isostéarylamine, la suif-amine et la soja-amine, (2) les amines secondaires correspondant à (1) ayant deux groupes identiques ou des mélanges de ces groupes, (3) les amines tertiaires correspondantes dans lesquelles tous le groupes dans le même molécule sont identiques ou différents ou (4) la N-octyl-1,2-éthylènediamine ou la N-octyl-1,3-propylènediamine, la N-coco-1,2-éthylènediamine ou la N-coco-1,3-propylènediamine, la N-oléyl-1,2- éthylènediamine ou la N-oléyl-1,3-propylènediamine, la N-soja-1,2-éthylènediamine ou la N-soja-1,3-propylènediamine, la N-suif-1,2-éthylènediamine ou la N-suif-1,3-propylènediamine, la N-éthyl-N-oléylamine, la N-méthyl-N-soja-amie, la N,N-diéthyl-N-oléylamine, la bis(2-hydroxyéthyl)-oléylamine, la bis(2-hydroxypropyl)-oléylamine, la bis(2-hydroxyéthyl)-sulfamine, la bis(2-hydroxypropyl)-suifamine, l'(hydroxyéthyl)-(hydroxypropyl)-suifamine, une oléylamine polyéthoxylée contenant 7 groupes éthoxy, une suifamine polyéthoxylée contenant 3 groupes éthoxy, des hydroalkylamines faites par éthoxylation ou propoxylation d'hydrocarbyldiamines ou d'hydrocarbyltriamines, la dodécyloxypropylamine ou la triisodécyloxypropylamine.

8. Une composition suivant l'une quelconque des revendications 1 à 6, caractérisée en ce que les entités _{D}hos_{D}hore et soufre sont fournies par un phosphorodithioate de formule dans laquelle R⁶ est un groupe hydrocarbyle contenant 3 à 18 atomes de carbone, M est un métal ou un non métal, n est la valence M et Z est un atome d'oxygène ou de soufre, l'un au moins des Z étant un atome de soufre.

9. Une composition suivant la revendication 8, caractérisée en ce que R⁶ est un groupe alkyle ou alkaryle.

10. Une composition suivant la revendication 9, caractérisée en ce que R⁶ est un groupe propyle, butyle, pentyle, hexyle, octyle, dodécyle, tétradécyle, tétradécyle, octadécyle, butylphényle, octylphényle, nonylphényle, dodécylphényle ou oléyle ou un mélange de ceux-ci.

11. Une composition suivant la revendication 10, caractérisée en ce que R⁶ dérive du propanol, de l'isopropanol, du butanol, de l'isobutanol, du sec-butanol, du 4-méthyl-2-pentanol, du 2-éthylhexanol et d'une mélange de ceux-ci.

12. Une composition suivant l'une quelconque des revendications 8 à 11, caractérisée en ce que le métal provient des Groupes IA, IIA, IIB et VIII du Tableau Périodique.

13. Une composition suivant la revendication 12, caractérisée en ce que le métal est le lithium, le molybdène, le sodium, le calcium, le zinc, le cadmium, l'argent ou l'or.

14. Une composition suivant l'une quelconqe des revendications 8 à 11, caractérisée en ce que M dérive de l'acétate de vinyle, du butyle vinyl éther, de l'oxyde de propylèné, du 1,2-époxydodécane ou d'un composé azoté.

15. Une composition suivant l'une quelconque des revendications 1 à 7, caractérisée en ce que les entités phosphore et soufre sont fournies par une combinaison comprenant (1) un phosphite de dihydrocarbyle ayant 2 à 10 atomes de carbone dans chaque groupe hydrocarbyle, des mélanges de phosphites ou un phosphate ayant 4 à 20 atomes de carbone dans chaque groupe hydrocarbyle et (2) un sulfure choisi parmi l'isobutylène sulfuré, le disulfure de dibenzyle, des terpènes sulfurés, le disulfire de phosphorodithionyle et une huile de jojoba sulfurée.

16. Une composition suivant la revendication 15, caractérisée en ce que le phosphite est un phosphite de dibutyle, dihexyle, dioctyle ou didécyle ou un mélang de ceux-ci.

17. Une composition suivant la revendication 15, caractérisée en ce que le phosphate est un phosphate de tributyle, tridécyle ou tricrésyle ou un mélange de ceux-ci.

18. Une composition suivant la revendication 1, caractérisée en ce que l'amine est la N-oléyl-1,3-propylènediamine, l'agent épaississant est un 12-hydroxystéarate et le phosphore et le soufre sont fournis par un alkyl (en C₃_₆)-phosphorodithioate de zinc.

19. Une composition suivant la revendication 1, caractérisée en ce que l'amine est la N-suif-1,3-propylènediamine, le composé du bore est l'acide borique l'agent épaississant est du 12-hydroxystéarate de lithium et les entités phosphore et soufre sont fournies par un alkyl(en C₃₋₆)-phosphorodithioate de zinc.

20. Une composition suivant l'une quelconque des revendications 1 à 19, caractérisée en ce que la graisse utilisée comme véhicule est une huile minérale.

21. Une composition suivant l'une quelconque des revendications 1 à 19, caractérisée en ce que la graisse utilisée comme véhicule est une huile synthétique.

22. Une composition suivant les revendications 20 et 21, caractérisée en ce que la graisse utilisée comme véhicule est un mélange d'huile synthétique et d'huile minérale.

23. Une composition suivant l'une quelconque des revendications 1 à 22, caractérisée en ce que la quantité totale d'agent épaississant est comprise entre environ 3 et 20% en poids de la composition total de graisse.

24. Procédé pour améliorer le point de goutte d'une composition de graisse comprenant une proportion majeure d'une graisse servant de véhicule et d'environ 0,01% à 10% en poids d'un produit de condensation obtenu par réaction d'un composé du bore avec une amine de formule: dans laquelle
x a une valeur de 0 à 2; R, R', R³ ou R⁴ représentent chacun un atome d'hydrogène ou un groupe hydrocarbyle en C₁₋₃₀, un groupe hydroxyalkyle en C₂₋₄, un groupe polyalcoxylé en C₆₋₂₀, ce dernier pouvant comprendre du soufre ou de l'oxygène supplémentaire, au moins l'un des R', R³ ou R⁴ n'étant pas un atome d'hydrogène et R² représente un groupe alkylène C_{Z}-₄, caractérisée en ce que cette graisse est épaissie avec un agent épaississant contenant au moins 15% en poids d'un savon contenant un substituant hydroxy en tant qu'agent épaississant.

25. Procédé suivant la revendication 24, caractérisé en ce que la composition de graisse contient de plus, d'environ 0,01% à 10% en poids d'un composé contenant à la fois du phosphore et du soufre ou un mélange de composés contenant du phosphore et contenant du soufre pour fournir une quantité équivalente de phosphore et de soufre.
